

3,161,584  
HYDROREFINING WITH DECOMPOSED  
ORGANO-METALLIC CATALYST

William K. T. Gleim, Island Lake, Ill., assignor to Universal Oil Products Company, Des Plaines, Ill., a corporation of Delaware  
No Drawing. Filed July 2, 1962, Ser. No. 207,070  
10 Claims. (Cl. 208—264)

This invention relates to a novel process for hydrorefining petroleum crude oils, heavy vacuum gas oils, heavy cycle stocks, etc., and to a novel catalyst especially adapted thereto. More specifically, the present invention involves a process for hydrorefining heavy hydrocarbon charge stocks to effect the removal of nitrogen and sulfur therefrom, and affords unexpected advantages when employed for the removal of metal contaminants and/or the conversion of pentane-insoluble asphaltenes into pentane-soluble hydrocarbon oils.

Crude petroleum oils, and also the heavier hydrocarbon fractions and/or distillate derived therefrom, generally contain considerable quantities of undesirable sulfurous and nitrogenous compounds. In addition, crude oils, and the heavy hydrocarbon fractions thereof, contain certain metallic contaminants which have an adverse effect on the activity of catalysts utilized in various processes to which crude oils, or heavy hydrocarbon fractions thereof, are ultimately subjected. The most common metallic contaminants are nickel and vanadium, although other metals including iron, copper, etc., are often present. These metals may occur in a variety of forms. They may exist as metal oxides or sulfides introduced into the crude oil as metallic scale or similar particles, or they may exist in the form of water-soluble salts of such metals. Usually however, they exist in the form of stable organometallic compounds, such as metal porphyrins and the various derivatives thereof.

Although the metallic contaminants existing in the form of an oxide or sulfide scale may be separated, at least in part, by relatively simple filtering techniques, and the water-soluble salts are at least in part removable by washing and subsequent dehydration, more extensive treatment is required to remove the stable organometallic compounds before the crude oil or heavy hydrocarbon charge is suitable for further processing.

In addition to organometallic compounds, crude oils contain greater quantities of sulfurous and nitrogenous compounds than are found in lighter hydrocarbon fractions such as gasoline, kerosene, light gas oil, etc. For example, a Wyoming sour crude, having a gravity of 23.2° API at 60° F., contains about 2.8% by weight of sulfur and about 2700 p.p.m. of total nitrogen. Reduction in the concentration of the sulfurous and nitrogenous compounds to the extent that the crude oil or heavy hydrocarbon charge is suitable for further processing, is accomplished with little difficulty by conversion to hydrogen sulfide and ammonia which are readily removed from the system in a gaseous phase. However, reduction in the concentration of the stable organometallic compounds to the extent that the crude oil or heavy hydrocarbon charge is suitable for further processing, is not as readily achieved. Notwithstanding that the concentration of these organometallic compounds is relatively small, for example, often less than about 10 p.p.m. calculated as the elemental metal, subsequent processing techniques are adversely affected thereby. For example, when a hydrocarbon charge stock containing metallic contaminants in excess of about 3 p.p.m. is subjected to catalytic cracking, the metals become deposited upon the catalyst, altering the composition thereof to the extent that undesirable by-products are formed. That is to say, the composition of the catalyst, which is closely con-

trolled with respect to the nature of the charge stock being processed and the quality and quantity of the product desired, is considerably changed as a result of the metal deposition thereon during the course of the cracking process. As a consequence the liquid product recovery is reduced, and coke and hydrogen are formed in excessive amounts, the former producing relatively rapid catalyst deactivation. The presence of organometallic compounds, including metal porphyrins, has an adverse effect on other processes including catalytic reforming, isomerization, hydrodealkylation, etc.

In addition, crude oils and other heavy hydrocarbon fractions generally contain large quantities of pentane-insoluble materials present in the form of a colloidal suspension or dispersion difficult to contact effectively with conventional hydrorefining catalysts. These pentane-insoluble materials, described as asphaltenes, are carbonaceous materials considered as coke precursors having a tendency to become immediately deposited within the reaction zone and on the catalytic composite as a gummy hydrocarbonaceous residue. It is further considered that said asphaltenes contain the bulk of the difficultly removable metal contaminants as well as a considerable portion of the undesirable nitrogenous and sulfurous compounds.

The object of the present invention is to provide a process for hydrorefining heavier hydrocarbonaceous materials, particularly petroleum crude oils, utilizing a catalyst formed in a particular manner. In other hydrorefining processes, the metals contained within the crude oil charge stock are removed therefrom by deposition of the same on the hydrorefining catalyst employed. This practice greatly increases the amount of catalyst in a relatively short time, precluding the use of a fixed-bed catalyst system commonly employed in present-day refining operations. Slurry processes, employing catalytically active metals deposited upon silica and/or alumina, are very erosive, and make plant upkeep difficult and expensive. The present invention teaches the preparation of a colloidally dispersed, unsupported catalyst useful in a slurry process, and which catalyst will not effect extensive erosion of the reaction system. The present process yields a liquid hydrocarbon product which is more suitable for further processing without experiencing the difficulties otherwise resulting from the presence of the above described contaminants. The process of the present invention is particularly advantageous in effecting the removal of organometallic compounds without significant product loss, while simultaneously converting pentane-insoluble materials into pentane-soluble liquid hydrocarbons.

In a broad embodiment, the present invention relates to a hydrorefining catalyst which comprises at least one decomposed xanthate complex of a metal of Groups VB, VIB, and the Iron group of the Periodic Table.

In another broad embodiment, the present invention encompasses a process of forming a hydrorefining catalyst which comprises forming a hydrocarbon solution of at least one xanthate complex of a metal of Groups VB, VIB, and the Iron group of the Periodic Table, and heating said solution at a temperature of less than about 310° C. for a time sufficient to decompose said xanthate complex.

The present invention involves a process for hydrorefining a hydrocarbon charge stock, which process comprises admixing said charge stock with at least one xanthate complex of a metal of Groups VB, VIB, and the Iron group of the Periodic Table, heating the resulting mixture at a temperature less than about 310° C. and for a time sufficient to decompose said xanthate complex, reacting the resulting colloidal suspension with hydrogen at a temperature in excess of about 225° C. and at a pres-

sure greater than about 500 pounds per square inch gauge, and recovering a hydrorefined liquid product.

More specifically, the present invention affords a process for hydrorefining a petroleum crude oil containing pentane-insoluble asphaltenes which comprises admixing said crude oil with molybdenum ethylxanthate, heating the resulting mixture at a temperature of less than about 310° C. for a time sufficient to decompose said molybdenum ethylxanthate, reacting the resulting colloidal suspension with hydrogen at a temperature of from about 225° C. to about 500° C. and at a pressure of from about 500 to about 5000 pounds per square inch gauge, and recovering said crude oil substantially free from pentane-insoluble asphaltenes.

From the foregoing embodiments it is readily ascertained that the process of the present invention involves the formation of a catalyst utilizing metals selected from Groups VB, VIB, and the Iron group of the Periodic Table (Handbook of Chemistry and Physics, 43rd ed.). The catalyst prepared in accordance with the method of the present invention, may comprise one or more metals from the group consisting of vanadium, niobium, tantalum, chromium, molybdenum, tungsten, iron, nickel, and cobalt. The catalyst is formed by initially dissolving a xanthate complex of the selected metal, or metals, in the hydrocarbon charge stock containing contaminating influences, including pentane-insoluble asphaltenes which are to be converted into soluble hydrocarbons. The quantity of a xanthate complex employed is such that said complex comprises from about 1.0 wt. percent to about 10.0 wt. percent of the hydrocarbon charge stock, calculated as the elemental metal. Suitable compounds which can be employed as a xanthate complex include niobium ethylxanthate, tantalum ethylxanthate, chromium ethylxanthate, iron ethylxanthate, nickel ethylxanthate, cobalt ethylxanthate, etc., and in particular vanadium methylxanthate, vanadium ethylxanthate, vanadium propylxanthate, vanadium isopropylxanthate, vanadium butylxanthate, vanadium isobutylxanthate, vanadium amylxanthate, vanadium isoamylxanthate, etc., and also molybdenum methylxanthate, molybdenum ethylxanthate, molybdenum propylxanthate, molybdenum isopropylxanthate, molybdenum butylxanthate, molybdenum isobutylxanthate, molybdenum amylxanthate, molybdenum isoamylxanthate, etc., and also tungsten methylxanthate, tungsten ethylxanthate, tungsten propylxanthate, tungsten isopropylxanthate, tungsten butylxanthate, tungsten isobutylxanthate, tungsten amylxanthate, tungsten isoamylxanthate, etc. The aforementioned xanthates, as well as other suitable xanthates, may be represented by the following general structural formula:



In the above structural formula, R can be a methyl, ethyl, or other alkyl group containing up to about 20 carbon atoms, the larger alkyl groups enhancing the oil solubility characteristics of the particular xanthate complex. R may also be an alkenyl, aryl, alkaryl, or aralkyl group. In the above formula, Me denotes a metal selected from the group consisting of vanadium, niobium, tantalum, chromium, molybdenum, tungsten, iron, nickel, and cobalt. In some instances, as in the case of the Group VB and VIB metals, Me is also representative of the metal in the form of an oxide thereof. For example, a molybdenum xanthate may be represented by the general formula illustrated below:



The xanthate complex of the selected metal may be prepared by any conventional or otherwise convenient

method. One suitable method comprises mixing an aqueous solution of the ammonium salt of the selected metal, for example ammonium molybdate, with an aqueous solution of an alkali metal xanthate, for example, potassium ethylxanthate. The resulting solution is neutralized with a weak acid, for example  $\text{SO}_2$ , to precipitate the desired xanthate complex. The precipitate is dried, and may be used as such or purified by recrystallization, for example, from benzene, alcohols, paraffins, etc.

The process is effected, as hereinabove set forth, by initially dissolving a desired quantity of the selected xanthate complex, for example molybdenum ethylxanthate, in the hydrocarbon charge stock. The xanthate complex may be added directly to the charge stock and dissolved therein. However, a preferred method comprises adding said xanthate complex as a solution thereof utilizing a suitable solvent such as an alcohol, benzene, and the like, while maintaining the charge stock at a temperature sufficient to distill the solvent therefrom substantially immediately as added. In either case the resulting mixture is then heated at a temperature less than about 310° C. for a time sufficient to effect decomposition of the xanthate complex, thereby forming the catalyst as a colloidal suspension, or dispersion, within the hydrocarbon charge stock. The decomposition of the xanthate complex is conducted at a temperature less than about 310° C. in order to avoid initial cracking of the petroleum crude oil prior to effecting complete decomposition of the xanthate complex.

The presence of free hydrogen during the above described decomposition procedure tends to have an adverse effect on catalyst activity with respect to the conversion of the pentane-insoluble fraction and removal of organometallic compounds. It is therefore preferred to exclude free hydrogen during said decomposition procedure. On the other hand, hydrogen sulfide appears to have a beneficial effect and its presence is preferred during the decomposition procedure as well as the subsequent hydrorefining procedure. The colloidal suspension or dispersion thus prepared is reacted with hydrogen at a temperature in excess of about 225° C., preferably at a temperature of from about 225° C. to about 500° C., and at a hydrogen pressure in excess of about 500 p.s.i.g., preferably at a pressure of from about 500 to about 5000 p.s.i.g.

This last mentioned treatment with hydrogen results in the conversion of a substantial portion of the pentane-insoluble asphaltenes to pentane-soluble hydrocarbons. In addition there is further formed what is herein referred to as a catalyst sludge which is readily separated from the hydrorefined product. Said catalytic sludge comprises unconverted asphaltenes, catalyst, and pentane-soluble hydrocarbons as well as the metal portion of the hydrocarbon charge stock separated therefrom. The process of this invention may be effected in any suitable

manner and may comprise either a batch or a continuous type of operation. For example, when a batch type of operation is employed, hydrogen and the hydrocarbon charge stock containing the colloidally dispersed catalyst are charged to an enclosed vessel and maintained therein at the desired temperature and pressure and with stirring. On completion of the hydrorefining process, the normally liquid hydrocarbons are separated from the reaction mixture by any suitable means, for example, through the use of a centrifuge or by means of a settling tank, the resulting catalyst sludge being recovered for re-use as such, or converted back to the xanthate complex by any of the well-known chemical means. The ammonia and hydrogen sulfide, resulting from the destructive conversion of sulfurous and nitrogenous compounds contained

70 within the petroleum crude oil, may be removed in a gaseous phase along with any light paraffinic hydrocarbons such as methane, ethane, and propane, etc. In a continuous type of operation, the starting materials, comprising hydrogen and the colloidal suspension, are continuously charged to a reactor maintained at the proper conditions

of temperature and pressure. The reaction mixture is continuously withdrawn from the reactor at a rate which will insure an adequate residence time therein. The hydrorefined product may be separated from the reactor effluent in the above described manner and the catalyst sludge recycled as a portion of the charge to the aforesaid reactor.

The following example will serve to further illustrate the process of this invention and the advantages to be derived therefrom with respect to separation of contaminating metals, pentane-insoluble asphaltenes, and nitrogenous and sulfurous compounds from the crude oil charge stock. It is not intended that the present invention be unduly limited to the catalyst, charge stock, and/or operating conditions employed within the example.

A Wyoming sour crude oil is utilized as a charge stock to illustrate the process of this invention. Such a charge stock has been found to contain about 2.8 wt. percent sulfur, approximately 2700 p.p.m. of nitrogen, 18 p.p.m. of nickel and 71 p.p.m. of vanadium as stable metal porphyrins, computed as the elemental metal. In addition, the sour crude contains 8.37 wt. percent pentane-insoluble asphaltenes. As hereinafter indicated, the process of the present invention effects the conversion of a substantial portion of said asphaltenes to the extent that the same no longer exert a detrimental effect on subsequent processing procedures.

A rotating steel autoclave of about 800 cc. capacity is utilized as a reaction vessel to illustrate the process of this invention. About 200 g. of the aforesaid crude oil and about 30 g. of molybdenum ethylxanthate are charged to the autoclave. The mixture is heated at about 250° C. to effect the decomposition of the molybdenum ethylxanthate, thus forming the catalyst as a colloidal suspension or dispersion in the crude oil. The autoclave is thereafter sealed, pressured with hydrogen, and heated at about 400° C. over about an 8 hour period. An initially imposed hydrogen pressure of about 100 atmospheres at about room temperature is suitable, rising to about 200 atmospheres at reaction temperature. At the expiration of the aforesaid 8 hour period, the autoclave contents are cooled and the autoclave is depressured. The reaction mixture is centrifuged and the supernatent liquid hydrocarbon product recovered. The liquid hydrocarbon, hydrorefined in the aforesaid manner, and will indicate less than about 0.5 wt. percent pentane-insoluble asphaltenes. In addition, there will be present less than about 100 p.p.m. of nitrogen, 0.10 wt. percent sulfur, 0.05 p.p.m. of nickel, 0.01 p.p.m. of vanadium.

The foregoing specifications and example will illustrate the advantages afforded the hydrorefining of petroleum crude oils due to utilization of the process of this invention. It is of particular interest to note that the nickel and vanadium porphyrin concentration, as well as the pentane-insoluble asphaltene concentration, is decreased to a level permitting subsequent utilization of the crude oil for further processing.

I claim as my invention:

1. A method of producing a catalyst which comprises forming a hydrocarbon solution of at least one xanthate complex of a metal selected from the group consisting of vanadium, niobium, tantalum, chromium, molybdenum, tungsten, iron, nickel and cobalt, and heating said solution at a temperature less than about 310° C. for a time sufficient to decompose said xanthate complex.

2. A process of claim 1 further characterized in that said xanthate complex comprises a xanthate complex of molybdenum.

3. A process for hydrorefining a hydrocarbon charge stock which comprises admixing said charge stock with at least one xanthate complex of a metal selected from the group consisting of vanadium, niobium, tantalum, chromium, molybdenum, tungsten, iron, nickel and cobalt, heating the resulting mixture at a temperature of less than about 310° C. and for time sufficient to decompose said xanthate complex, reacting the resulting colloidal suspension with hydrogen at a temperature in excess of about 225° C. and at a pressure greater than about 500 pounds per square inch gauge, and recovering a hydrorefined liquid product.

4. The process of claim 3 further characterized in that the colloidal suspension of said charge stock and decomposed xanthate complex is reacted with hydrogen at a temperature of from about 225° C. to about 500° C. and under an imposed pressure of from about 500 to about 5000 pounds per square inch gauge.

5. The process of claim 3 further characterized in that said xanthate complex is a xanthate complex of molybdenum.

6. A process for hydrorefining a petroleum crude oil containing pentane-insoluble asphaltenes which comprises admixing said crude oil with at least one xanthate complex of a metal selected from the group consisting of vanadium, niobium, tantalum, chromium, molybdenum, tungsten, iron, nickel and cobalt, heating the resulting mixture at a temperature less than about 310° C. and for a time sufficient to decompose said xanthate complex, reacting the resulting colloidal suspension with hydrogen at a temperature in excess of about 225° C. and at a pressure greater than about 500 pounds per square inch gauge, and recovering said crude oil substantially free of pentane-insoluble asphaltenes.

7. The process of claim 6 further characterized in that said xanthate complex is decomposed within said crude oil in a non-reducing atmosphere.

8. The process of claim 6 further characterized in that the mixture of said crude oil and decomposed xanthate complex is reacted with hydrogen in the absence of carbon monoxide.

9. The process of claim 8 further characterized in that said xanthate complex is a xanthate complex of molybdenum.

10. A process for hydrorefining a petroleum crude oil containing pentane-insoluble asphaltenes which comprises admixing said crude oil with molybdenum ethylxanthate heating the resulting mixture at a temperature of less than about 310° C. for a time sufficient to decompose said molybdenum ethylxanthate, reacting the resulting colloidal suspension with hydrogen at a temperature of from about 22° C. to about 500° C. and at a pressure of from about 500 to about 5000 pounds per square inch gauge and recovering said crude oil substantially free of pentane-insoluble asphaltenes.

References Cited in the file of this patent

UNITED STATES PATENTS

- 2,999,075      Pruett ----- Sept. 5, 196  
3,053,756      Nottes et al. ----- Sept. 11, 196